

## UNITED STATES PATENT OFFICE

2,689,195

PROCESS FOR TREATING SYNTHETIC  
TEXTILES

John Donald Martone, Wilmington, Del., assignor  
to E. I. du Pont de Nemours and Company,  
Wilmington, Del., a corporation of Delaware

No Drawing. Application January 31, 1952,  
Serial No. 269,343

10 Claims. (Cl. 117—65)

**1**  
This invention relates to a method for treating textiles composed of polymers and copolymers of acrylonitrile. More particularly, it relates to a process for treating textiles such as the filaments, fibers, yarns, staple, fabrics, and the like, of polymers and copolymers of acrylonitrile to permit uniform darkening when they are exposed to an elevated temperature.

It is a matter of common knowledge that textiles, such as the filaments, fibers, yarns, staple, fabrics, and the like, produced from polymers and copolymers of acrylonitrile darken when they are exposed to an elevated temperature. Furthermore, it has been observed that this darkening is not uniform. In the case of fabrics, warp streaks, filling barré, and the like result, which in many instances destroy the commercial value of the material. The temperatures experienced upon exposure to the weather, as for instance upon awnings, auto tops, and the like, as well as those due to frictional sources, as upon machinery drive belts, and the like, have been found to produce the unsightly effect.

It is an object of this invention to provide a process for the treatment of textiles such as filaments, fibers, yarns, staple, fabrics, and the like, of polymers and copolymers of acrylonitrile which will eliminate the variable darkening tendency on exposure to an elevated temperature.

A further object is to produce a textile such as a filament, fiber, yarn, staple, fabric, or the like, of polymers and copolymers of acrylonitrile which darkens uniformly on exposure to an elevated temperature.

These and other objects will become apparent in the course of the following specification and claims.

The objects of the present invention are accomplished by subjecting the textile such as the filament, fiber, yarn, staple, fabric, or the like, to a treatment comprising the following steps:

1. Scouring, with or without a suitable detergent, to remove size, finish material or other substances with which the textile has been coated.

2. Boiling-off in an aqueous solution of a low molecular weight aliphatic carboxylic acid containing minor amounts of a sulfate of a long chain aliphatic alcohol.

3. Rinsing with soft water to remove traces of acid.

After such treatment, the textile of polymers or copolymers of acrylonitrile may be subjected to an elevated temperature without streaking due to non-uniform darkening.

**2**

The following example is cited by way of illustration and not by way of limitation.

*Example*

A swatch 12" x 12", woven in a 90 x 82 construction, taffeta pattern from 100 denier continuous filament polyacrylonitrile yarn which contains a coating of gelatin as a size, is scoured in a bath containing 0.2% of the sodium sulfate of commercial lauryl alcohol as a detergent. At the end of 30 minutes, the swatch is boiled-off (212° F.) for two hours in an aqueous solution containing 2% oxalic acid and 0.2% of a commercial mixture of a sodium sulfate of commercial lauryl alcohol. The swatch is then rinsed with soft water until free of residual acid. Thereafter, the fabric is air dried at a temperature of approximately 180° F.

Upon subjecting the swatch to a temperature of 350° F. for 3 1/3 minutes, the material darkened appreciably. However, this darkening is uniform, free from filling barré, warp streaks, and the like.

When a swatch of the same material is subjected to heat in accordance with the conditions of the procedure outlined above, without the pre-treatment described, a non-uniform darkening is observed showing pronounced short length variations, warp streaks and filling barré.

By a textile of polymer of acrylonitrile is meant the filament, fiber, yarn, staple, fabric, and the like, produced by extrusion of polymerized acrylonitrile, such as is illustrated in United States Patent No. 2,404,714 to Latham dated July 23, 1946. Furthermore, copolymers of acrylonitrile, wherein the acrylonitrile comprises about 35% or more are likewise suitable. Among the copolymerizable compounds which may be mentioned as being suitable are methyl methacrylate, vinyl acetate, methyl vinyl ketone, vinyl pyridine, etc. Such copolymeric materials and others are shown in United States Patents Nos. 2,436,926 to Jacobson, dated March 2, 1948, and 2,491,471 to Arnold, dated December 20, 1949.

While the example cited above illustrates the use of oxalic acid as the low molecular weight aliphatic carboxylic acid, other such water-soluble organic acids may be used as well. Among these may be mentioned formic, propionic and acetic. Oxalic acid is preferred since it appears to give optimum results under the conditions outlined. Acid concentrations will vary somewhat, depending on the acid. A 1% to 2% solution has been found effective for oxalic acid.

The sulfate of the long chain aliphatic alcohol may be any of such alcohols containing from 10 to 18 carbon atoms. Among these may be mentioned decyl, dodecyl, cetyl, lauryl, oleyl and the like. Furthermore, mixtures of such materials may be used. Thus, alcohols prepared by the hydration of alkenes formed in the cracking of petroleum are suitable. A trace of this material is sufficient. Normally, 0.1 to 0.2% is employed.

The treatment described is effective for all physical forms of textiles of polymers or copolymers of acrylonitrile. It is likewise applicable to all types of woven or knitted fabric, whether formed from continuous monofilament or multifilament yarn or from spun yarn of staple or from mixtures of these yarns. While the invention is primarily concerned with fabrics of polymers or copolymers of acrylonitrile, it is also useful and advantageous in the handling of fabrics made from mixed yarns wherein the polyacrylonitrile element is admixed with one or more other natural or synthetic element such as nylon or wool.

The nature of the detergent in the first step is not critical. Its choice will be governed by the particular type of size or finish which has been previously applied by design or accident. Thus, as the example illustrates, where a gelatin starch size has been employed, it has been found convenient to use the sodium sulfate of commercial lauryl alcohol as detergent. However, any suitable anionic, cationic or non-ionic detergent may be used. Soap is frequently sufficient. The period of scouring will be governed by the type of finish and the effectiveness of the detergent used.

The boiling-off step in the presence of organic acid and aliphatic alcohol sulfate is usually accomplished by immersing the fabric in a jig which is held at the boiling temperature of the mixture. This is not essential, however, and the solution may be applied to the textile in other ways, such as by a beck scour or the like, provided sufficient contact at the proper temperature is maintained. The period of contact will vary widely depending upon the nature of the treating agents and their concentrations within the aqueous solution. It has been found that even at the lower concentrations, a period of one hour is usually sufficient. Longer periods of treatment are sometimes desirable. No deleterious effects result from extended periods of contact.

The rinsing step can be accomplished by any conventional method, such as immersion, spraying, or the like. The wash water may be removed by wringing, if desired, to facilitate the drying operation. The drying may be accomplished in an air drier or oven provided the heat is not in excess of 300° F.

While the specific example has been drawn to the pretreatment of a fabric prior to exposure to an elevated temperature, it is obvious that the process is applicable as well to pretreatment of filaments, fibers, yarns, staple, and the like. Many other modifications within the spirit of the disclosed invention will be apparent to those skilled in the art without a departure from the inventive concept.

What is claimed is:

1. A process for the treatment of a textile com-

prising a member of the group consisting of polymers and copolymers of acrylonitrile prior to exposure to elevated temperatures which comprises the steps of scouring the textile, contacting it for a period of about one hour with a boiling aqueous solution of a low molecular weight aliphatic carboxylic acid containing a minor amount of a sulfate of a long chain aliphatic alcohol and rinsing with water.

2. The process of claim 1 wherein the low molecular weight aliphatic carboxylic acid is oxalic acid.

3. A process for the treatment of a polyacrylonitrile fiber which comprises the steps of scouring the fiber, contacting it for a period of about one hour with a boiling aqueous solution of oxalic acid containing a minor amount of a long chain aliphatic alcohol of from ten to eighteen carbon atoms and rinsing with water.

4. The process of claim 3 wherein the sulfate of the long chain aliphatic alcohol is the sulfate of a mixture prepared by the hydration of alkenes formed in the cracking of petroleum.

5. The process of claim 3 wherein the sulfate of the long chain aliphatic alcohol is the sulfate of lauryl alcohol.

6. A process for the treatment of a textile comprising a member of the group consisting of polymers and copolymers of acrylonitrile prior to exposure to elevated temperature which comprises the steps of scouring the said textile in the presence of a detergent, immersing it for at least about an hour in boiling water containing from about 0.1 to about 0.2% of a sulfate of an aliphatic alcohol containing from ten to eighteen carbon atoms and from about 1 to about 2% of a low molecular weight aliphatic carboxylic acid and thereafter rinsing the said textile with water.

7. The process of claim 6 wherein the textile is a fabric.

8. The process of claim 7 wherein the acid is oxalic and the alcohol is lauryl alcohol.

9. A process for the treatment of a polyacrylonitrile textile which comprises the steps of scouring the said textile for about 30 minutes in a bath containing about 0.2% of a detergent, thereafter immersing the said textile in boiling water containing about 2% oxalic acid and 0.2% of sodium lauryl sulfate for a period of about 2 hours, rinsing the said textile with soft water until free of residual acid and thereafter drying in air at a temperature of about 180° F.

10. The process of claim 9 wherein the textile is thereafter uniformly darkened by subjecting it to a temperature of about 350° C. for about 3 minutes.

References Cited in the file of this patent  
UNITED STATES PATENTS

|           |                |               |
|-----------|----------------|---------------|
| Number    | Name           | Date          |
| 2,404,357 | Bechtold ----- | July 23, 1946 |
| 2,431,956 | Moody -----    | Dec. 2, 1947  |

FOREIGN PATENTS

|         |              |               |
|---------|--------------|---------------|
| Number  | Country      | Date          |
| 905,038 | France ----- | Nov. 22, 1945 |